

1,069,791.

A. C. KRUEGER.

STORAGE CELL.

APPLICATION FILED AUG. 1, 1912.

Patented Aug. 12, 1913.

Fig. 5.



Fig. 4.



Fig. 3.



Fig. 1.



Fig. 2.



Witnesses:

Harry Krueger  
Henry Klippel.

Inventor:

August C. Krueger

# UNITED STATES PATENT OFFICE.

AUGUST C. KRUEGER, OF MILWAUKEE, WISCONSIN.

## STORAGE-CELL.

1,069,791.

Specification of Letters Patent. Patented Aug. 12, 1913.

Application filed August 1, 1912. Serial No. 712,653.

To all whom it may concern:

Be it known that I, AUGUST C. KRUEGER, a citizen of the United States, residing at 745 Hubbard street, Milwaukee, in the 5 county of Milwaukee and State of Wisconsin, have invented a new and useful Storage-Cell, of which the following is a specification.

My invention relates to storage cells, by 10 means of which—as commonly understood—electrical energy is stored for future use.

The objects are, to furnish a storage cell of higher efficiency and greater power, but 15 less liable to injurious chemical action, than any other known today. To attain these objects I use antimony electrodes and a saturated hydrochloric acid solution of compounds of antimony and chlorin, preferably antimony trichlorid, as the electrolyte. By 20 using these, equally good results may be obtained regardless of any one particular design or construction of the cell, providing the general rules and principles, pertaining to storage battery engineering, are observed. 25 Hence I do not limit myself to the precise construction, as illustrated in the accompanying drawing and herein following description thereof, wherein—

Figure 1 is a vertical section of the entire 30 storage cell, as indicated by the dotted line C—C in Fig. 2, which is a top view of the cell; Fig. 3 is a cross section through the entire cell, as indicated by the dotted line B—B in Fig. 1; Fig. 4 is a full size section 35 of part of one of the twenty-four antimony plates P, that constitute the electrodes, showing that part which slides over the connecting rods S' or S, and part of the grooved surface; Fig. 5 is a cross section of the cup-shaped upper part of the glass rod L, as indicated by the dotted line A—A in Fig. 1.

The containing vessel O is made of glass, and has three circular cavities in the bottom 40 to hold the two antimony connecting rods S' S and the glass rod L in place, as illustrated in Fig. 1; the cover K is also of glass and firmly screwed to the containing vessel O by means of the six bolts N.

The twelve antimony plates, that 50 constitute the positive electrode, are connected and held together in a horizontal position, by sliding one above the other onto the antimony rod S', interposed by the twelve antimony plates that constitute the similarly 55 constructed negative electrode with the anti-

mony rod S, as illustrated in Fig. 1; the glass rings R (marked in Fig. 3 only) separate the positive and negative plates from each other, and also serve as supports for them. In the center, through the plates and 60 rings, is placed the glass rod L, which terminates at the top in a cup form, so as to permit the funnel-shaped extension in the center of the cover K to slide into it, thus holding it in place and preventing the plates 65 and rings from shifting; J' J Q I are rubber bands.

The glass stopper F can be removed by releasing the brass spring G, for the purpose 70 of filling the cell with the electrolyte; the four holes M, as illustrated in Fig. 5, permit the liquid to pass through as indicated by the two arrows in Fig. 1; the dotted line E—E indicates the proper height for the 75 electrolyte.

The binding posts D' D are of brass, and 80 form the terminals of the cell; they are screwed to the antimony caps H' H, into the two circular holes in the cover K; the antimony rods S' S connect with the antimony caps H' H by sliding into them when the glass cover K is screwed in place, thus forming complete connections, as illustrated in Fig. 1.

Each antimony plate is perforated with 85 sixteen holes, as illustrated in Fig. 3, to allow a more free circulation in the electrolyte. To offer a good surface for effective electrolytical action, the plates are grooved on both sides in a checkered manner, as illustrated in Fig. 3 and Fig. 4. The two tubes 90 of antimony T' T are for the purpose of holding down more firmly the plates that constitute the electrodes.

The following is my theory of the chemical reactions that seem to take place during 95 charge and discharge: Before the actual charging commences an initial current is applied to dissociate the water in the solution, 100 causing partial oxidation of the positive electrode. Then the current is reversed and the following reactions take place:

### At the Negative Plates.

During charge:



During discharge:



*At the Positive Plates.*

During charge:



5 During discharge:



The functions of the antimony chlorid in the electrolyte, I can not fully define, but 10 can merely say that it increases the conductivity of the electrolyte.

I claim:

The combination, in a storage cell, of antimony electrodes, and an electrolyte containing chlorids of hydrogen and antimony, substantially as specified. 15

AUGUST C. KRUEGER.

Witnesses:

HARRY KRUEGER,  
HENRY KLIPPEL.

Copies of this patent may be obtained for five cents each, by addressing the "Commissioner of Patents, Washington, D. C."